

## UNITED STATES PATENT OFFICE.

CHRISTIAN I. GILLSTRAP, OF CRYSTAL LAKE, IOWA.

## FUEL AND PROCESS OF MAKING SAME.

No Drawing.

Application filed February 23, 1921. Serial No. 447,231.

*To all whom it may concern:*

Be it known that I, CHRISTIAN I. GILLSTRAP, a citizen of the United States, residing at Crystal Lake, in the county of Hancock and State of Iowa, have invented new and useful Improvements in Fuel and Processes of Making Same, of which the following is a specification.

This invention relates to fuel and has for its object the provision of a process for converting lignite, bituminous, sub-bituminous, and various types of lignitic matter into coke suitable for use in any art or in any capacity.

It is well known in the art that lignite is ordinarily useless, or at least practically so as it cannot be coked under any of the usual methods owing to the fact that it crumbles. It is with this fact in view that the present invention has been designed. The present invention has for its primary object the provision of a process by which material of this nature may be properly coked so as to form a fuel which may be used for any and all purposes.

In carrying out my invention I take a suitable quantity, for instance one ton, of lignite, sub-bituminous coal, or other lignitic matter, crushed to a sufficient fineness so as to pass through a one inch mesh screen, and add to it twenty pounds, more or less, of pitch or coal tar which has been melted so as to be poured over the crushed lignite or coal. I also mix with this mass one hundred pounds of clay, such as ordinary clay, or clay containing a variable amount of iron pyrites. I also add forty pounds, more or less, of ground commercial coke which is preferably crushed so as to pass through an inch screen. This entire mixture is heated in a coke oven and maintained at a temperature varying from five hundred to a thousand degrees centigrade for six hours, during which time all the moisture is expelled from the mixture and all the volatile matter from the coal is driven off. It is of course intended that this volatile matter be caught and condensed so that the valuable by-products may be saved.

The carrying out of my process is very simple as there is enough gas expelled from

the mixture during the heating thereof to furnish the heat for coking ovens, there being consequently no waste of fuel in the operation. The clay found overlying the lignite coal beds of North Dakota, Montana, Wyoming, and Texas is well suited for use in my process. The volatile matter expelled during the coking of the mixture will, when condensed, provide the necessary tar to act as the binder.

From experience I have discovered that the coke produced by my process is a highly efficient fuel adapted for all purposes, and that it burns freely and leaves little ash and no clinker or slag.

While I have enumerated the proportions of the ingredients used I desire to have it distinctly understood that the proportions and specific character of the ingredients may be varied and that the temperature used in effecting the coking may be varied considerably. Neither do I limit myself to any exact size of coal as I have found that coal of various sizes will coke by my process, and on account of the excess moisture in lignite coal I have found it necessary to crush it to various sizes depending on the moisture in it so as to have it give up all the moisture evenly during the process. It is also to be understood that I reserve the right to make any changes in the carrying out of my process which will come within the scope of the subjoined claims.

Having thus described my invention, I claim:

1. The process of forming artificial fuel consisting in grinding lignitic material, adding ground clay, ground commercial coke and a tar binder thereto, and subsequently coking the mixture by subjecting it to a temperature of from 500° to 1000° centigrade.

2. An artificial fuel consisting of a mixture of 2000 parts of crushed lignitic material, 20 parts of coal tar, 100 parts of ground clay, and 40 parts of ground commercial coke mixed together and heated to effect coking.

In testimony whereof I hereto affix my signature.

CHRIS GILLSTRAP,